

[54] ELECTROPHOTORESISTIVE MATERIALS FOR MIGRATION IMAGING PROCESSES

[75] Inventors: James R. Nonnemacher, Rochester; Michael T. Regan, Fairport; Frank G. Webster, Rochester, all of N.Y.

[73] Assignee: Eastman Kodak Company, Rochester, N.Y.

[21] Appl. No.: 909,245

[22] Filed: May 24, 1978

[51] Int. Cl.<sup>2</sup> ..... G03G 13/24

[52] U.S. Cl. ..... 96/1 PE; 96/1.3; 96/1.5 R

[58] Field of Search ..... 96/1 PE, 1.3, 1.5 R

[56] References Cited

U.S. PATENT DOCUMENTS

- |           |         |                  |                  |
|-----------|---------|------------------|------------------|
| 2,328,652 | 9/1943  | Kirby et al.     | ..... 96/56.2    |
| 3,384,566 | 5/1968  | Clark            | ..... 96/1 PE    |
| 3,630,749 | 12/1971 | Webster et al.   | ..... 96/140     |
| 3,719,480 | 3/1973  | Brantly          | ..... 96/1.5 R X |
| 3,721,554 | 3/1973  | Nagashima et al. | ..... 96/1.5 R   |
| 3,743,638 | 7/1973  | Webster et al.   | ..... 260/240.4  |
| 3,900,318 | 8/1975  | Zographos et al. | ..... 96/1 PE X  |
| 3,912,507 | 10/1975 | Keller et al.    | ..... 96/1.5 R   |
| 3,961,952 | 6/1976  | Sprague          | ..... 96/1.5 R   |
| 4,012,376 | 3/1977  | Wright           | ..... 96/1.5 R X |
| 4,017,311 | 4/1977  | Gruber           | ..... 96/1.3 X   |

FOREIGN PATENT DOCUMENTS

- |         |        |                |              |
|---------|--------|----------------|--------------|
| 1018110 | 1/1966 | United Kingdom | ..... 96/1.5 |
|---------|--------|----------------|--------------|

Primary Examiner—Roland E. Martin, Jr.  
Attorney, Agent, or Firm—John R. Everett

[57]

ABSTRACT

Electrophotoreactive materials having the structure



wherein

R represents a basic heterocyclic nucleus as well as groups such as hydrogen, alkyl, aryl, aralkyl, etc.;

A<sub>1</sub> represents a wide variety of basic heterocyclic nuclei;

A<sub>2</sub> represents aryl or may be the same as A<sub>1</sub>;

G represents O or S;

M is 0 to 3;

N is 0 to 1; and

L<sup>1</sup>, L<sup>2</sup>, L<sup>3</sup>, L<sup>4</sup> and L<sup>5</sup> represent hydrogen, alkyl or aryl.

4 Claims, 1 Drawing Figure



FIG. 1



## ELECTROPHOTOSENSITIVE MATERIALS FOR MIGRATION IMAGING PROCESSES

### FIELD OF THE INVENTION

This invention relates to electrophoretic migration imaging processes and, in particular, to the use of certain novel photosensitive pigment materials in dispersions for such processes.

### BACKGROUND OF THE INVENTION

In the past, there has been extensive description in the patent and other technical literature of electrophoretic migration imaging processes. For example, a description of such processes may be found in U.S. Pat. No. 2,758,939 by Sugarman issued Aug. 14, 1956; U.S. Pat. Nos. 2,940,847, 3,100,426, 3,140,175 and 3,143,508, all by Kaprelian; U.S. Pat. Nos. 3,384,565, 3,384,488 and 3,615,558, all by Tulagin et al; U.S. Pat. No. 3,384,566 by Clark; and 3,383,993 by Yeh. In addition to the foregoing patents directed to conventional photoelectrophoretic migration imaging processes, another type of electrophoretic migration imaging process which advantageously provides for image reversal is described in Groner, U.S. Pat. No. 3,976,485 issued Aug. 24, 1976. This latter process is called photoimmobilized electrophoretic recording or PIER.

In general, each of the foregoing electrophoretic migration imaging processes employs a layer of electrostatic charge-bearing photoconductive particles, i.e., 30 electrically photosensitive particles, positioned between two spaced electrodes, one of which may be transparent. To achieve image formation in these processes, the charge-bearing photosensitive particles positioned between the two spaced electrodes, are subjected to the 35 influence of an electric field and exposed to activating radiation. As a result, the charge-bearing electrically photosensitive particles are caused to migrate electro- 40 phoretically to the surface of one or the other of the spaced electrodes, and one obtains an image pattern on 45 the surface of these electrodes. Typically, a negative image is formed on one electrode, and a positive image is formed on the opposite electrode. Image discrimination occurs in the various electrophoretic migration imaging processes as a result of a net change in charge 50 polarity of either the exposed electrically photosensitive particles (in the case of conventional electrophoretic migration imaging) or the unexposed electrically photosensitive particles (in the case of the electrophoretic migration imaging process described in the above-noted Groner patent) so that the image formed on one electrode surface is composed ideally of electrically photosensitive particles of one charge polarity, either negative or positive polarity, and the image formed on the opposite polarity electrode surface is composed ideally of electrically photosensitive particles having the opposite charge polarity, either positive or negative respectively.

In any case, regardless of the particular electrophoretic migration imaging process employed, it is apparent that an essential component of any such process is the electrically photosensitive particles. And, of course, to obtain an easy-to-read, visible image it is important that these electrically photosensitive particles be colored, as well as electrically photosensitive. Accordingly, there 65 exists a continuing effort to find particles which possess both useful levels of electrical photosensitivity and which exhibit good colorant properties. Thus, various

types of electrically photosensitive materials are disclosed for use in electrophoretic migration imaging processes, for example, in U.S. Pat. Nos. 2,758,939 by Sugarman, 2,940,847 by Kaprelian, and 3,384,488 and 3,615,558 by Tulagin et al., noted hereinabove.

Up to now, useful electrically photosensitive or photoconductive pigment materials for electrophoretic migration imaging have been selected from known classes of photoconductive materials which may be 10 employed in conventional photoconductive elements, e.g., photoconductive plates, drums, or webs used in electrophotographic office-copier devices. For example, both Sugarman and Kaprelian in the above-referenced patents state that electrically photosensitive materials useful in electrophoretic migration imaging processes may be selected from known classes of photoconductive materials. Also, the phthalocyanine pigments described as a useful electrically photosensitive material for electrophoretic imaging processes in U.S. Pat. No. 3,615,558 by Tulagin et al. have long been known to exhibit useful photoconductive properties.

### SUMMARY OF THE INVENTION

The present invention provides a group of materials which are useful in electrophoretic migration imaging dispersions, images and processes. To the best of our knowledge, none of said materials have been previously identified as photoconductors. The materials of this invention have one of the following structures:



wherein:

R represents any one of a wide variety of basic heterocyclic nuclei such as defined for A<sup>1</sup> below and may also represent groups such as hydrogen, and the following may be further substituted alkyl, aryl, aralkyl, ureido, thioureido, hydroxy, anilino, amidino, etc. Said substituents may be groups such as alkoxy, aryloxy, hydroxy, carboxy, cyano, halogens, alkoxy carbonyl, etc.

G represents O or S;

L<sup>1</sup>, L<sup>2</sup>, L<sup>3</sup>, L<sup>4</sup>, and L<sup>5</sup>, each represent hydrogen, alkyl, or aryl;

M represents zero, one, two or three;

N represents zero or one;

A<sup>1</sup> represents a nitrogen substituted basic heterocyclic nucleus of the type used in cyanine dyes. Such dyes include:

- (a) imidazole, such as 4-phenylimidazole;
- (b) 3H-indole nucleus such as 3H-indole, 3,3-dimethyl-3H-indole, 3,3,5-trimethyl-3H-indole;
- (c) a thiazole nucleus such as thiazole, 4-methylthiazole, 5-phenylthiazole, 5-methylthiazole, 5-phenylthiazole, 4,5-dimethylthiazole, 4,5-diphenylthiazole, and 4-(2-thienyl)thiazole;
- (d) a benzothiazole nucleus such as benzothiazole, 5-aminobenzothiazole, 4-chlorobenzothiazole, 5-chlorobenzothiazole, 6-chlorobenzothiazole, 5-cyanobenzothiazole, 4-methylbenzothiazole, 5-methylbenzothiazole, 6-bromobenzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, tetrahydrobenzothiazole, 5,6-dimethoxybenzothiazole, 5,6-methylenedioxobenzothiazole, 5-hydroxybenzothiazole and 6-hydroxybenzothiazole;
- (e) a naphthothiazole nucleus such as naphtho[1,2-d]thiazole, naphtho[2,1-d]thiazole, naphtho[2,3-d]thiazole, 5-methoxynaphtho[2,1-d]thiazole, 5-ethoxynaphtho[2,1-d]thiazole, 8-methoxynaphtho[1,2-d]thiazole, 7-methoxynaphtho[1,2-d]thiazole and 4,5-dihydroneaphtho[1,2-d]thiazole;
- (f) a thianaphtheno[7,6-d]thiazole nucleus such as 4-methoxythianaphtheno[7,6-d]thiazole;
- (g) an oxazole nucleus such as 4-methyloxazole, 5-methyloxazole, 4-phenyloxazole, 4,5-diphenyloxazole, 4-ethyloxazole, 4,5-dimethyloxazole and 5-phenyloxazole;
- (h) a benzoxazole nucleus such as benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 5-ethoxybenzoxazole, 6-chlorobenzoxazole, 6-methoxybenzoxazole, 5-hydroxybenzoxazole and 6-hydroxybenzoxazole;
- (i) a naphthoxazole nucleus such as naphth[1,2-d]oxazole, naphth[2,1-d]oxazole and naphth[2,3-d]oxazole;
- (j) a selenazole nucleus such as 4-methylselenazole and 4-phenylselenazole;
- (k) a benzoselenazole nucleus such as benzoselenazole, 5-chlorobenzoselenazole, 5-methoxybenzoselenazole, 5-hydroxybenzoselenazole and tetrahydrobenzoselenazole;
- (l) a naphthoselenazole nucleus such as naphtho[1,2-d]selenazole, naphtho[2,1-d]selenazole;
- (m) a thiazoline nucleus such as thiazoline and 4-methylthiazoline;
- (n) a 2-quinoline nucleus such as quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, and 8-hydroxyquinoline;
- (o) a 4-quinoline nucleus such as quinoline, 6-methoxyquinoline, 7-methylquinoline and 8-methylquinoline;
- (p) a 1-isoquinoline nucleus such as isoquinoline and 3,4-dihydroisoquinoline;
- (q) a benzimidazole nucleus such as 1-ethylbenzimidazole and 1-phenylbenzimidazole;
- (r) a 2-pyridine nucleus such as pyridine and 5-methylpyridine; and
- (s) a 4-pyridine nucleus.

Ring nitrogen substituents on the above basic heterocyclic nuclei may be alkyl, aryl, and aralkyl which may be further substituted by groups such as alkoxy, aryloxy, alkoxycarbonyl, acyl, hydroxy, cyano, amino, alkylamino, arylamino, dialkylamino, diarylamino, halogens, etc.

$A^2$  may represent the same basic heterocyclic nucleus as  $A^1$  and in addition may represent an amino substituted aryl group (e.g., p-aminophenyl) or an alkoxy substituted aryl group (e.g., 4-methoxyphenyl, 1-methoxy-2-naphthyl, or 1-ethoxy-2-anthryl) or  $A^2$  may be for example, a heterocyclic nucleus such as thiophene, benzo[b]thiophene, naphtho[2,3-b]thiophene, furan, isobenzofuran, chromene, pyran, xanthene, pyrrole, 2H-pyrrole, pyrazole, indolizine, indoline, indole, indazole, carbazole, pyrimidine, isothiazole, isoxazole, furazan, chroman, isochroman, 1,2,3,4-tetrahydroquinoline, 4H-pyrrolo [3,2,1-ij]quinoline, 1,2-dihydro-4H-pyrrolo[3,2,1-ij]quinoline; 1,2,5,6-tetrahydro-4H-pyrrolo[3,2,1-ij]quinoline; 1H,5H-benzo[ij]quinolizine; 2,3-dihydro-1H,5H-benzo[ij]quinolizine; 2,3-dihydro-1H,5H-benzo[ij]quinolizine and 2,3,6,7-tetrahydro-1H,5H-benzo[ij]quinolizine, 10,11-dihydro-9H-benzo[a]xanthan-8-yl; 6,7-dihydro-5H-benzo[b]pyran-7-yl.

Unless stated otherwise, alkyl refers to aliphatic hydrocarbon groups of generally 1-20 carbon atoms such as methyl, ethyl, propyl, isopropyl, butyl, heptyl, dodecyl, octadecyl and eicosyl, etc. Aryl refers to aromatic ring groups of 6-20 carbons such as phenyl, naphthyl, anthryl or to alkyl or aryl substituted aryl groups such as tolyl, ethylphenyl, biphenyl, etc. Aralkyl refers to aryl substituted alkyl groups where aryl and alkyl are as described above e.g., benzyl, phenethyl. Alkoxy refers to groups  $RO^-$  where R is alkyl as described above.

When used in an electrophoretic migration imaging process, charge-bearing, electrically photosensitive particles formulated from the materials of the present invention are positioned between two spaced electrodes.

40 While so positioned between the spaced electrodes, the photosensitive particles are subjected to an electric field and exposed to a pattern of activating radiation. As a consequence, the charge-bearing, electrically photosensitive particles undergo a radiation-induced variation in their charge polarity and migrate to one or the other of the electrode surfaces to form on at least one of these electrodes an image pattern representing a positive-sense or negative-sense image of the original radiation exposure pattern.

#### BRIEF DESCRIPTION OF THE DRAWINGS

The FIGURE represents diagrammatically a typical imaging apparatus for carrying out the electrophoretic migration imaging process of the invention.

#### DESCRIPTION OF THE PREFERRED EMBODIMENTS

A preferred embodiment of the present invention provides a group of materials which are useful in electrophoretic migration imaging dispersions and processes, and have the structure of Formulas I & II wherein:

$L^1$ ,  $L^2$ ,  $L^3$ ,  $L^4$ ,  $L^5$ ,  $M$ ,  $N$ ,  $R$ , and  $G$  are as previously defined;

65  $A^1$  represents a nitrogen substituted basic heterocyclic nucleus such as 3H-indole, benzothiazole, naphthothiazole, benzoxazole, benzoselenazole, 2-quinoline, 4-quinoline and thiazoline; and

$A^2$  represents dialkylaminophenyl.

A more preferred embodiment of the present invention provides a group of materials which are useful in electrophoretic migration imaging processes which have the structure of Formulas I and II wherein:

R represents hydrogen, methyl, ethyl, naphthyl, thioureido, phenyl, benzothiazolyl, hydroxy, anilino and amidino;

G represents O;

$L^1$ ,  $L^2$ ,  $L^3$ ,  $L^4$ , and  $L^5$ , represent hydrogen or methyl;

M represents one or two;

N represents one;

$A^1$  represents 3H-indole, naphtho[1,2-d]thiazole, 4,5-dihydronephtho[1,2-d]thiazole; benzoxazole, benz-selenazole, 2-quinoline, 4-quinoline and thiazoline with 15 alkyl substituents on the ring nitrogen; and

$A^2$  represents dimethylaminophenyl.

In general, the materials of Formulas I & II which have been found to be electrophotosensitive tend to exhibit a maximum absorption wavelength,  $\delta_{max}$ , within the range of from about 420 to about 750 nm. A variety of different materials within the class defined by Formula I have been tested and found to exhibit useful levels of electrical photosensitivity in electrophoretic migration imaging processes.

A partial listing of representative such materials is included herein in Table I. Materials included in Formulas I & II may be prepared according to the procedures set out in U.S. Pat. Nos. 2,328,652 and 3,743,638. Structurally similar materials are disclosed as spectral sensitizers for silver halide emulsions in U.S. Pat. No. 3,630,749.

TABLE I

| Number | Material | Color        |
|--------|----------|--------------|
| 1      |          | Purple       |
| 2      |          | Red          |
| 3      |          | Orange       |
| 4      |          | Brownish Red |
| 5      |          | Purple       |

TABLE I-continued

| Number | Material | Color         |
|--------|----------|---------------|
| 6      |          | Orange        |
| 7      |          | Red           |
| 8      |          | Purple        |
| 9      |          | Purple        |
| 10     |          | Purple        |
| 11     |          | Yellow        |
| 12     |          | Reddish Brown |

TABLE I-continued

| Number | Material | Color   |
|--------|----------|---------|
| 13     |          | Magenta |
| 14     |          | Purple  |
| 15     |          | Purple  |
| 16     |          | Purple  |
| 17     |          | Purple  |
| 18     |          | Purple  |

TABLE I-continued

| Number | Material | Color   |
|--------|----------|---------|
| 19     |          | Green   |
| 20     |          | Orange  |
| 21     |          | Blue    |
| 22     |          | Purple  |
| 23     |          | Orange  |
| 24     |          | Magenta |
| 25     |          | Orange  |

TABLE I-continued

| Number | Material                                                                          | Color  |
|--------|-----------------------------------------------------------------------------------|--------|
| 26     |  | Purple |
| 27     |  | Purple |

The electrically photosensitive material described herein is useful in the preparation of the electrically photosensitive imaging particles and dispersions used in electrophoretic migration imaging processes. In general, electrically photosensitive particles useful in such processes have an average particle size within the range of from about 0.01 micron to about 20 microns, preferably from about 0.01 to about 5 microns. Typically, these particles are composed of one or more colorant materials such as the colorant materials described in the present invention. However, these electrically photosensitive particles may also contain various nonphotosensitive materials such as electrically insulating polymers, charge control agents, various organic and inorganic fillers, as well as various additional dyes or pigment materials to change or enhance various colorant and physical properties of the electrically photosensitive particle. In addition, such electrically photosensitive particles may contain other photosensitive materials such as various sensitizing dyes and/or chemical sensitizers to alter or enhance their response characteristics to activating radiation.

When used in an electrophoretic migration imaging process in accord with the present invention, the electrically photosensitive material described in Table I is typically positioned in particulate form, between two or more spaced electrodes, one or both of which typically are transparent to radiation to which the electrically photosensitive material is light-sensitive, i.e., activating radiation. Although the electrically photosensitive material, in particulate form, may be dispersed simply as a dry powder between two spaced electrodes and then subjected to a typical electrophoretic migration imaging operation such as that described in U.S. Pat. No. 2,758,939 by Sugarman, it is more typical to disperse the electrically photosensitive particulate material in an electrically insulating carrier, such as an electrically insulating liquid, or an electrically insulating, liquefiable matrix material, such as a heat- and/or solvent-softenable polymeric material or a thixotropic polymeric material. Typically, when one employs such a dispersion of electrically photosensitive particulate material and electrically insulating carrier material between the spaced

electrodes of an electrophoretic migration imaging system, it is conventional to employ from about 0.05 part to about 2.0 parts of electrically photosensitive particulate material for each 10 parts by weight of electrically insulating carrier material.

As indicated above, when the electrically photosensitive particles used in the present invention are dispersed in an electrically insulating carrier material, such carrier material may assume a variety of physical forms and may be selected from a variety of different materials. For example, the carrier material may be a matrix of an electrically insulating, normally solid polymeric material capable of being softened or liquefied upon application of heat, solvent, and/or pressure so that the electrically photosensitive particulate material dispersed therein can migrate through the matrix. In another, more typical embodiment of the invention, the carrier material can comprise an electrically insulating liquid such as decane, paraffin, Sohio Odorless Solvent 3440 (a kerosene fraction marketed by the Standard Oil Company, Ohio), various isoparaffinic hydrocarbon liquids such as those sold under the trademark Isopar G by Exxon Corporation and having a boiling point in the range of 145° C. to 186° C., various halogenated hydrocarbons such as carbon tetrachloride, trichloromonofluoromethane, and the like, various alkylated aromatic hydrocarbon liquids such as the alkylated benzenes, for example, xylenes, and other alkylated aromatic hydrocarbons such as are described in U.S. Pat. No. 2,899,335. An example of one such useful alkylated aromatic hydrocarbon liquid which is commercially available is Solvesso 100 made by Exxon Corporation. Solvesso 100 has a boiling point in the range of about 157° C. to about 177° C. and is composed of 9 percent dialkyl benzenes, 37 percent trialkyl benzenes, and 4 percent aliphatics. Typically, whether solid or liquid at normal room temperatures, i.e., about 22° C., the electrically insulating carrier material used in the present invention is a material having a resistivity greater than about 10<sup>9</sup> ohm-cm, preferably greater than about 10<sup>12</sup> ohm-cm. When the electrically photosensitive particles formed from the materials of the present invention are incorporated in a

carrier material, such as one of the above-described electrically insulating liquids, various other addenda may also be incorporated in the resultant imaging suspension. For example, various charge control agents may be incorporated in such a suspension to improve the uniformity of charge polarity of the electrically photosensitive particles dispersed in the liquid suspension. Such charge control agents are well known in the field of liquid electrographic developer compositions where they are employed for purposes substantially similar to that described herein. Thus, extensive discussion of the materials herein is deemed unnecessary. These materials are typically polymeric materials incorporated by admixture thereof into the liquid carrier vehicle of the suspension. In addition to, and possibly related to, the aforementioned enhancement of uniform charge polarity, it has been found that the charge control agents often provide more stable suspensions, i.e., suspensions which exhibit substantially less settling out of the dispersed photosensitive particles.

In addition to the foregoing charge control agent materials, various polymeric binder materials such as various natural, semi-synthetic or synthetic resins, may be dispersed or dissolved in the electrically insulating carrier to serve as a fixing material for the final photosensitive particle image formed on one of the spaced electrodes used in electrophoretic migration imaging systems. Here again, the use of such fixing addenda is conventional and well known in the closely related art of liquid electrographic developer compositions so that extended discussion thereof is unnecessary herein.

The process of the present invention will be described in more detail with reference to the accompanying drawing, FIG. 1, which illustrates a typical apparatus which employs the electrophoretic migration imaging process of the invention.

FIG. 1 shows a transparent electrode 1 supported by two rubber drive rollers 10 capable of imparting a translating motion via original image 11 to electrode 1 in the direction of the arrow. Electrode 1 may be composed of a layer of optically transparent material, such as glass or an electrically insulating, transparent polymeric support such as polyethylene terephthalate, covered with a thin, optically transparent, conductive layer such as tin oxide, indium oxide, nickel, and the like. Optionally, depending upon the particular type of electrophoretic migration imaging process desired, the surface of electrode 1 may bear a "dark charge exchange" material, such as a solid solution of an electrically insulating polymer and 2,4,7,trinitro-9-fluorenone as described by Groner in U.S. Pat. No. 3,976,485 issued Aug. 24, 1976.

Spaced opposite electrode 1 and in pressure contact therewith is a second electrode 5, an idler roller which serves as a counter electrode to electrode 1 for producing the electric field used in the electrophoretic migration imaging process. Typically, electrode 5 has on the surface thereof a thin, electrically insulating layer 6. Electrode 5 is connected to one side of the power source 15 by switch 7. The opposite side of the power source 15 is connected to electrode 1 so that as an exposure takes place, switch 7 is closed and an electric field is applied to the electrically photosensitive particulate material 4 which is positioned between electrodes 1 and 5. Typically, electrically photosensitive particulate material 4 is dispersed in an electrically insulating carrier material such as described hereinabove.

The electrically photosensitive particulate material 4 may be positioned between electrodes 1 and 5 by apply-

ing material 4 to either or both of the surfaces of electrodes 1 and 5 prior to the imaging process or by injecting electrically photosensitive imaging material 4 between electrodes 1 and 5 during the electrophoretic migration imaging process.

As shown in FIG. 1, exposure of electrically photosensitive particulate material 4 takes place by use of an exposure system consisting of light source 8, an original image 11 to be reproduced, such as a photographic transparency, a lens system 12, and any necessary or desirable radiation filters 13, such as color filters, whereby electrically photosensitive material 4 is irradiated with a pattern of activating radiation corresponding to original image 11. Although the electrophoretic migration imaging system represented in FIG. 1 shows electrode 1 to be transparent to activating radiation from light source 8, it is possible to irradiate electrically photosensitive particulate material 4 in the nip 21 between electrodes 1 and 5 without either of electrodes 1 or 5 being transparent. In such a system, although not shown in FIG. 1, the exposure source 8 and lens system 12 is arranged so that image material 4 is exposed in the nip or gap 21 between electrodes 1 and 5.

As shown in FIG. 1, electrode 5 is a roller electrode having a conductive core 14 connected to power source 15. The core is in turn covered with a layer of insulating material 6, for example, baryta paper. Insulating material 6 serves to prevent or at least substantially reduce the capability of electrically photosensitive particulate material 4 to undergo a radiation induced charge alteration upon interaction with electrode 5. Hence, the term "blocking electrode" may be used, as is conventional in the art of electrophoretic migration imaging, to refer to electrode 5.

Although electrode 5 is shown as a roller electrode and electrode 1 is shown as essentially a translatable, flat transparent plate electrode in FIG. 1, either or both of these electrodes may assume a variety of different shapes such as a web electrode, rotating drum electrode, opaque plate electrode, and the like as is well known in the field of electrophoretic migration imaging. In general, during a typical electrophoretic migration imaging process wherein electrically photosensitive material 4 is dispersed in an electrically insulating, liquid carrier, electrodes 1 and 5 are spaced such that they are in pressure contact or very close to one another during the electrophoretic migration imaging process, e.g., less than 50 microns apart. However, where electrically photosensitive particulate material 4 is dispersed simply in an air gap between electrodes 1 and 5 or in a carrier such as a layer of heat-softenable or other liquefiable material coated as a separate layer on electrode 1 and/or 5, these electrodes may be spaced more than 50 microns apart during the imaging process.

The strength of the electric field imposed between electrodes 1 and 5 during the electrophoretic migration imaging process of the present invention may vary considerably; however, it has generally been found that optimum image density and resolution are obtained by increasing the field strength to as high a level as possible without causing electrical breakdown of the carrier medium in the electrode gap. For example, when electrically insulating liquids such as isoparaffinic hydrocarbons are used as the carrier in the imaging apparatus of FIG. 1, the applied voltage across electrodes 1 and 5 typically is within the range of from about 100 volts to about 4 kilovolts or higher.

As explained hereinabove, image formation occurs in electrophoretic migration imaging processes as the result of the combined action of activating radiation and electric field on the electrically photosensitive particulate material 4 disposed between electrodes 1 and 5 in the attached drawing. Typically, for best results, field application and exposure to activating radiation occur concurrently. However, as would be expected, by appropriate selection of various process parameters such as field strength, activating radiation intensity, incorporation of suitable light sensitive addenda in or together with the electrically photosensitive particles formed from the material of Formula I, e.g., by incorporation of a persistent photoconductive material, and the like, it is possible to alter the timing of the exposure and field application events so that one may use sequential exposure and field application events rather than concurrent field application and exposure events.

When disposed between imaging electrodes 1 and 5 of FIG. 1, electrically photosensitive particulate material 4 exhibits an electrostatic charge polarity, either as a result of triboelectric interaction of the particles or as a result of the particles interacting with the carrier material in which they are dispersed, for example, an electrically insulating liquid, such as occurs in conventional liquid electrographic developing compositions composed of toner particles which acquire a charge upon being dispersed in an electrically insulating carrier liquid.

Image discrimination occurs in the electrophoretic migration imaging process of the present invention as a result of the combined application of electric field and activating radiation on the electrically photosensitive particulate material dispersed between electrodes 1 and 5 of the apparatus shown in FIG. 1. That is, in a typical imaging operation, upon application of an electric field between electrodes 1 and 5, the particles 4 of charge-bearing, electrically photosensitive material are attracted in the dark to either electrodes 1 or 5, depending upon which of these electrodes has a polarity opposite to that of the original charge polarity acquired by the electrically photosensitive particles. And, upon exposing particles 4 to activating electromagnetic radiation, it is theorized that there occurs neutralization or reversal of the charge polarity associated with either the exposed or unexposed particles. In typical electrophoretic migration imaging systems wherein electrode 1 bears a conductive surface, the exposed, electrically photosensitive particles 4, upon coming into electrical contact with such conductive surface, undergo an alteration (usually a reversal) of their original charge polarity as a result of the combined application of electric field and activating radiation. Alternatively, in the base of photoimmobilized electrophoretic recording (PIER), wherein the surface of electrode 1 bears a dark charge exchange material as described by Groner in aforementioned U.S. Pat. No. 3,976,485, one obtains reversal of the charge polarity of the unexposed particles, while maintaining the original charge polarity of the exposed electrically photosensitive particles, as these particles come into electrical contact with the dark charge exchange surface of electrode 1. In any case, upon the application of electric field and activating radiation to electrically photosensitive particulate material 4 disposed between electrodes 1 and 5 of the apparatus shown in FIG. 1, one can effectively obtain image discrimination so that an image pattern is formed by the electrically photosensitive particles which correspond

to the original pattern of activating radiation. Typically, using the apparatus shown in FIG. 1, one obtains a visible image on the surface of electrode 1 and a complementary image pattern on the surface of electrode 5.

Subsequent to the application of the electric field and exposure to activating radiation, the images which are formed on the surface of electrodes 1 and/or 5 of the apparatus shown in FIG. 1 may be temporarily or permanently fixed to these electrodes or may be transferred to a final image receiving element. Fixing of the final particle image can be effected by various techniques, for example, by applying a resinous coating over the surface of the image bearing substrate. For example, if electrically photosensitive particles 4 are dispersed in a liquid carrier between electrodes 1 and 5, one may fix the image or images formed on the surface of electrodes 1 and/or 5 by incorporating a polymeric binder material in the carrier liquid. Many such binders (which are well known for use in liquid electrophotographic liquid developers) are known to acquire a charge polarity upon being admixed in a carrier liquid and therefore will, themselves, electrophoretically migrate to the surface of one or the other of the electrodes. Alternatively, a coating of resinous binder (which has been admixed in the carrier liquid), may be formed on the surfaces of electrodes 1 and/or 5 upon evaporation of the liquid carrier.

The electrically photosensitive colorant material of Formulas I & II may be used to form monochrome images, or the material may be admixed with other electrically photosensitive material of proper color and photosensitivity and used to form polychrome images. Many of the electrically photosensitive colorant materials having Formulas I & II have especially useful hues which make them particularly suited for use in polychrome imaging processes which employ a mixture of two or more differently colored electrically photosensitive particles. When such a mixture of multicolored electrically photosensitive particles is formed, for example, in an electrically insulating carrier liquid, this liquid mixture of particulate material exhibits a black coloration. Preferably, the specific cyan, magenta, and yellow particles selected for use in such a polychrome imaging process are chosen so that their spectral response curves do not appreciably overlap whereby color separation and subtractive multicolor image reproduction can be achieved.

The following examples illustrate the utility of the Formula I materials in electrophoretic migration imaging processes.

#### EXAMPLES 1-27

##### Imaging Apparatus

An imaging apparatus was used in each of the following examples to carry out the electrophoretic migration imaging process described herein. This apparatus was a device of the type illustrated in FIG. 1. In this apparatus, a translating film base having a conductive coating of 0.1 optical density cermet (Cr.SiO) served as electrode 1 and was in pressure contact with a 10 centimeter diameter aluminum roller 14 covered with dielectric paper coated with poly(vinyl butyral) resin which served as electrode 5. Plate 1 was supported by two 2.8 cm. diameter rubber drive rollers 10 positioned beneath film plate 1 such that a 2.5 cm. opening, symmetric with the axis of the aluminum roller 14, existed to allow exposure of electrically photosensitive particles 4 to

activating radiation. The original transparency 11 to be reproduced was taped to the back side of film plate 1.

The original transparency to be reproduced consisted of adjacent strips of clear (W0), red (W29), green (W99) and blue (W47B) filters. The light source consisted of a Kodak Ektographic AV434A Carousel Projector with a 1000 watt Xenon Lamp. The light was modulated with a Kodak No. 5 flexible M-carbon eleven step 0.3 neutral density step tablet. The residence time in the action or exposure zone was 10 milliseconds. The log of the light intensity (Log I) was as follows:

| Filters | Log I |                           |
|---------|-------|---------------------------|
|         |       | erg/cm <sup>2</sup> /sec. |
| W0      | Clear | 5.34                      |
| W29     | Red   | 4.18                      |
| W99     | Green | 4.17                      |
| W47B    | Blue  | 4.15                      |

The voltage between the electrode 5 and film plate 1 was about 2 kv. Film plate 1 was negative polarity in the case where electrically photosensitive particulate material 4 carried a positive electrostatic charge, and film plate 1 was positive in the case where electrically photosensitive electrostatically charged particles were negatively charged. The translational speed of film plate 1 was about 25 cm. per second. In the following examples, image formation occurs on the surfaces of film plate 1 and electrode 5 after simultaneous application of light exposure and electric field to electrically photosensitive material evaluated for use. Electrically photosensitive particulate material 4 was admixed with a liquid carrier as described below to form a liquid imaging dispersion which was placed in nip 21 between the electrodes 1 and 5. If the material being evaluated for use as material 4 possessed a useful level of electrical photosensitivity, one obtained a negative-appearing image reproduction of original 11 on electrode 5 and a complementary image on electrode 1.

#### Imaging Dispersion Preparation

Imaging dispersions were prepared to evaluate each of the materials in Table I. The dispersions were prepared by first making a stock solution of the following components. The stock solution was prepared simply by combining the components.

Isopar G—2.2 g  
Solvesso—1.3 g  
Piccotex 100—1.4 g

PVT\*—0.1 g

\*Poly(vinyltoluene-co-lauryl methacrylate-co-lithium methacrylate-co-methacrylic acid) 56/40/3.6/0.4

A 5 g. aliquot of the stock solution was combined in a closed container with 0.045 g. of the Table I material to be tested and 12 g. of Pioneer 440 stainless steel balls. The preparation was then milled for three hours on a paint shaker.

Each of the 27 materials described in Table I were tested according to the just outlined procedures. Each of such materials was found to be electrophotosensitive as evidenced by obtaining a negative appearing image of the original on one electrode and a complementary image on the other electrode. Materials 1, 2, 3, 4, 6, 7, 9, 11, 12, 14, 15, 17, 18, 20, 21, 22, 24, 26 and 27 provide images having good to excellent quality. Image quality was determined visually having regard to minimum and maximum densities, speed and color saturation.

The invention has been described in detail with particular reference to certain preferred embodiments thereof, but it will be understood that variations and modifications can be effected within the spirit and scope of the invention.

We claim:

1. An electrophoretic migration imaging process which comprises subjecting an electrically photosensitive colorant material positioned between at least two electrodes to an applied electric field and exposing said materials to an image pattern of radiation to which the material is photosensitive, thereby obtaining image formation on at least one of said electrodes, characterized in that at least a portion of said material is an electrically photosensitive material having one of the following structures:



I.



wherein:

R represents a basic heterocyclic nucleus of the type described from A<sup>1</sup> below, hydrogen, alkyl, aryl, aralkyl, ureido, thioureido, hydroxy, anilino or amidino;

G represents O or S;

L<sup>1</sup>, L<sup>2</sup>, L<sup>3</sup>, L<sup>4</sup>, and L<sup>5</sup>, each represent hydrogen, alkyl, or aryl;

M represents zero, one, two or three;

N represents zero or one;

A<sup>1</sup> represents a basic nitrogen substituted heterocyclic nucleus selected from the group consisting of imidazole, 3H-indole, thiazole, benzothiazole, naphthothiazole, thianaphtheno[7,6-d]thiazole, oxazole, benzoxazole, naphthoxazole, selenazole, benzoselenazole, naphthoselenazole, thiazoline, 2-quinoline, 4-quinoline, 1-isoquinoline, benzimidazole, 2-pyridine and 4-pyridine;

A<sup>2</sup> may represent the same basic heterocyclic nucleus as A<sup>1</sup> and in addition may represent an amino substituted aryl group or an alkoxy substituted aryl group or A<sup>2</sup> may be for example, a heterocyclic nucleus such as thiophene, benzo[b]thiophene, naphtho[2,3-b]thiophene, furan, isobenzofuran, chromene, pyran, xanthene, pyrrole, 2H-pyrrole, pyrazole, indolizine, indoline, indole, indazole, carbazole, pyrimidine, isothiazole, isoxazole, furazan, chroman, isochroman, 1,2,3,4-tetrahydroquinoline, 4H-pyrrolo[3,2,1-ij]quinoline, 1,2-dihydro-4H-pyrrolo[3,2,1-ij]quinoline; 1,2,5,6-tetrahydro-4H-pyrrolo[3,2,1-ij]quinoline; 1H,5H-ben-

zo[ij]quinolizine; 2,3-dihydro-1H,5H-benzo[ij]-quinolizine; 2,3-dihydro-1H,5H-benzo[ij]quinolizine and 2,3,6,7-tetrahydro-1H,5H-benzo[ij]quinolizine, 10,11-dihydro-9H-benzo[a]xanthene-5-yl; 6,7-dihydro-5H-benzo[b]pyran-7-yl.

**2. A process according to claim 1, wherein:**

$L^1, L^2, L^3, L^4, L^5, M, N, R$  and  $Y$  are as previously defined:

$A^1$  represents a nitrogen substituted 3H-indole, benzothiazole, naphthothiazole, benzoxazole, benzoselenazole, 2-quinoline, 4-quinoline or thiazoline; and  $A^2$  represents dimethylaminophenyl.

3. An electrophoretic migration imaging process which comprises subjecting an electrically photosensitive colorant material positioned between at least two electrodes to an applied electric field and exposing said materials to an image pattern of radiation to which the material is photosensitive, thereby obtaining image formation on at least one of said electrodes, characterized in that at least a portion of said material is an electrically photosensitive material having one of the following structures: 20 25



**wherein:**

R represents hydrogen, methyl, ethyl, naphthyl, thioureido, phenyl, benzothiazolyl, hydroxy, anilino and amidino; 50

**G represents O:**

$L^1, L^2, L^3, L^4$ , and  $L^5$  represent hydrogen or methyl: 55

M represents one or two:

N represents one:

**A<sup>1</sup>** represents a nitrogen substituted 3,3-dimethyl-3H-indole, naphtho[1,2-d]-thiazole, 4,5-dihydronaphtho[1,2-d]thiazole; benzoxazole, benzoselenazole, 2-quinoline, 4-quinoline or thiazoline; and

$\Delta^2$  represents dimethylaminophenyl

4. A process according to claim 3 wherein at least a portion of said material is an electrically photosensitive material having one of the following structures: 65



-continued



-continued



\* \* \* \* \*

UNITED STATES PATENT AND TRADEMARK OFFICE  
CERTIFICATE OF CORRECTION

PATENT NO. 4,165,985

DATED August 28, 1979

INVENTOR(S) James R. Nonnemacher et al

It is certified that error appears in the above-identified patent and that said Letters Patent are hereby corrected as shown below:

Column 7, No. 7, change "



Column 7, No. 11, change "



Signed and Sealed this

First Day of January 1980

[SEAL]

Attest:

SIDNEY A. DIAMOND

Attesting Officer

Commissioner of Patents and Trademarks